

## UNITED STATES PATENT OFFICE

DANIEL LAGRANGE AND FERDINAND DE PAPE, OF UCCLE, BELGIUM, ASSIGNORS TO  
LA SOUDURE ELECTRIQUE AUTOGÈNE SOCIÉTÉ ANONYME, OF BRUSSELS, BELGIUM

## FUSIBLE ELECTRODE FOR ELECTRIC WELDING

No Drawing. Application filed May 28, 1930, Serial No. 456,802, and in France June 6, 1929.

This invention relates to the electrodes used in welding by the electric arc and has for its object the provision of an electrode for welding aluminium, copper, iron, steel, etc., which will enable the special properties of the welded metal to be improved, especially as regards mechanical resistance.

According to the invention, the composition of the covering for the core contains beryllium. It is well known that relatively small proportions of beryllium alloyed with copper, aluminium, etc., increase the rupture stress and the hardness (Brinell) of these metals. Also, beryllium hardens iron considerably; 2 to 4% of beryllium increases its hardness up to about 300 and more. It is further known to add usual alloying metals for iron, copper, etc., in the coating with or without a reducing agent.

It has now been found that by adding beryllium in the coating of the metallic core of an electrode, an alloy containing beryllium is smoothly and evenly deposited by the welding operation, and that furthermore the normal working voltage is reduced through a particularly favorable ionization of the arc interval. It has never been proposed to use beryllium in the coatings of electrodes, as an alloying metal for the metallic core, although in a general way it has been proposed to add alloying metals such as chromium or vanadium, etc., by including these alloying metals, for instance, in the coating of an electrode, to obtain as weld metal the corresponding alloy without, however, the smooth welding and reduced voltage obtained when beryllium is used as in the invention.

According to the invention, electrodes for welding copper or aluminium or their alloys can be coated, for instance, by a suitable flux, forming a saline coating such as described in the U. S. patent application, No. 319,023, filed November 12, 1928, since matured into Patent No. 1,888,453, dated November 22, 1932, and divisional application, No. 482,916, filed September 18, 1930, since matured into Patent No. 1,898,427, dated February 21, 1933, both in the name of Ferdinand de Pape, and with powdered metallic beryllium

or a beryllium compound incorporated in the coating with eventually a known reducing agent such as carbon. For instance, fluosilicate or beryllium can be added to said coating without a reducing agent, while carbon should be added to oxide of beryllium to obtain a deposit free from metallic oxides. An electrode according to the invention and intended specially to obtain deposits of great hardness, for instance, in casehardening iron or steel (e. g., rails, gearing, etc.), consists of a rod of soft iron combined with a coating containing beryllium or a beryllium compound with or without a reducing agent. The metallic beryllium or beryllium compounds are usually added to the coating in proportions varying from 0.25% to 30% in weight of the dry coating. These are not, however, fast limits to the scope of the invention.

When a relatively great percentage of beryllium is to be alloyed with the iron, copper, or aluminium, the core of the electrode can be made out of a corresponding beryllium alloy, coated with a coating containing beryllium or a beryllium compound. The coating may, for instance, be obtained as follows; 80 grammes of active carbon are caused to absorb 100 cubic centimeters of beryllium chloride in a 99% solution. After more or less thorough drying, the product obtained is treated with concentrated ammonia. By this means beryllium hydrate is precipitated in the pores of the active carbon, the product is washed in water, to remove the greater part of the ammonium chloride formed, and then subjected to a slight calcination to expel the rest of the ammonium chloride. The calcined product is ground and added to the coating composed as mentioned, in proportions varying from 5 to 25% in weight of the dry coating, to cover a copper rod or a copper alloy rod.

In the same way, in the composition of salt coatings, for aluminium or aluminium alloy electrodes, according to this latter method of carrying out the invention, a chloride or other suitable compound of beryllium may be used, in suitable propor-

tions, in one or the other stages of the examples of the processes which are the object of the described United States patent applications No. 319,023, filed November 12, 1928, 5 and No. 482,916, filed September 18, 1930, both in the name of Ferdinand de Pape.

A coating is thus obtained consisting of a fluosilicated compound, containing beryllium compounds, of which the greater part 10 is reduced by the action of the electric welding arc.

We claim:

1. An electrode for electric arc welding comprising a metallic core and a coating on 15 the core, said electrode containing by weight of the core from 0.25% to 30% of beryllium.

2. An electrode for electric arc welding comprising a metallic core and a coating on the core, said electrode containing in the 20 coating and by weight of the core from 0.25% to 30% of finely-divided metallic beryllium.

3. An electrode for electric arc welding comprising a metallic core and a coating 25 on the core, said electrode containing in the coating and by weight of the core from 0.25% to 30% of beryllium in the form of a beryllium alloy.

4. An electrode for electric arc welding 30 comprising a metallic core and a coating on the core, said electrode containing in the coating and by weight of the core from 0.25% to 30% of beryllium in the form of a beryllium compound.

35 5. An electrode for electric arc welding

comprising a copper core and a coating on the core, said electrode containing in the coating from 0.25% to 30% of beryllium by weight of the core.

6. An electrode for electric arc welding 70 comprising an aluminum core and a coating on the core, said electrode containing in the coating from 0.25% to 30% of beryllium by weight of the core.

7. An electrode for electric arc welding 75 comprising an iron core and a coating on the core, said electrode containing in the coating from 0.25% to 30% of beryllium by weight of the core.

8. An electrode for electric arc welding 80 comprising a core consisting of a copper-beryllium alloy and a coating on the core containing beryllium, said electrode containing from 0.25% to 30% beryllium by weight of the core.

9. An electrode for electric arc welding comprising a core consisting of an aluminum-beryllium alloy and a coating on the core containing beryllium, said electrode containing from 0.25% to 30% beryllium by 90 weight of the core.

10. An electrode for electric arc welding comprising a core consisting of an iron-beryllium alloy and a coating on the core containing beryllium, said electrode containing from 0.25% to 30% beryllium by weight of the core.

DANIEL LAGRANGE.  
FERDINAND DE PAPE.

40

105

45

110

50

115

55

120

60

125

65

130